

# UNITED STATES PATENT OFFICE.

CHARLES G. OSBORNE, OF CHICAGO, ILLINOIS.

## PROCESS OF TREATING MANGANESE-STEEL INGOTS.

1,094,090.

Specification of Letters Patent. Patented Apr. 21, 1914.

No Drawing.

Application filed March 5, 1913. Serial No. 752,240.

*To all whom it may concern:*

Be it known that I, CHARLES G. OSBORNE, a citizen of the United States, residing at Chicago, in the county of Cook and State 5 of Illinois, have invented certain new and useful Improvements in Processes of Treating Manganese-Steel Ingots, of which the following is a specification.

My invention relates to improvements in 10 the manufacture of manganese steel ingots, and refers particularly to the process of heat treatment of such ingots and the product resulting therefrom.

It is well known that when an ingot of 15 manganese steel containing approximately 9 to 16% of manganese and .80 to 1.40% of carbon is allowed to cool slowly, either in an ingot mold or by being freely exposed to the air, a layer of weakly adhering dendrites is formed at temperatures below approximately 1150° centigrade, these dendrites forming to a greater extent as the steel approaches the temperature of recrystallization, which may be roughly taken as 20 600 to 800° centigrade, but which is generally not above 750° centigrade, at which temperatures of recrystallization the ingot acquires a coarse crystalline structure. By 25 heating an ingot to a temperature of approximately 1150-1215° C., the dendrites are gradually broken up, and an interlocking structure takes the place of the columnar dendritic structure. When this result is accomplished, the ingot is ready for rolling. 30 It will be apparent that the lower the temperature is to which the ingot cools slowly the longer will be the time required in order to break up the dendritic structure on reheating. Thus the maximum time is 35 required when the ingot cools to or below its temperature of recrystallization, whereas, on the other hand, when the ingot is placed into a soaking pit before its temperature has fallen below approximately 1150° C., 40 the time required is only that which is necessary to equalize the temperature of the interior and exterior of the ingot, since there has been only at the most a slight formation of dendrites.

It is the object of my invention to treat 45 manganese steel ingots so that if it is necessary to allow them to cool the reheating may be effected in a much less time than has heretofore been necessary. I accomplish 50 this result by quenching the ingot at as high a temperature as is possible, thereby rapidly

cooling the steel to a temperature at which structural changes no longer take place and preventing an excessive formation of dendrites, and, as it were, holding the steel with 60 the same structure which it had at the temperature at which it was quenched. It will now be evident that when an ingot is reheated for rolling it will be unnecessary to break up an excessive dendritic structure, 65 since by means of the quenching the formation of this structure has been prevented.

In carrying out my invention, the ingot is preferably quenched as soon after it has been stripped as is practicable.

It will be apparent that by my invention a great economy in time and fuel is obtained.

Where an ingot is taken directly to the soaking pit after it has been stripped it is unnecessary to use my process, since the reheating begins before the temperature of the ingot has fallen sufficiently to allow the excessive formation of dendrites. If, on the other hand, operating conditions necessitate delays and the cooling of the ingot, my process should be employed, and the ingot quenched in water or other suitable fluid as soon after stripping as is possible. Similarly, in the case of overheated ingots, which are ordinarily impossible to roll or forge, I 75 have found that by quenching such ingots their original structure seems to be restored, and they may then be reheated and rolled or forged without difficulty.

It will be apparent to those skilled in the 80 art that changes could be made in the exact invention which I have described without departing from its spirit or scope.

What I claim is:

1. The process of treating a cast body of 85 manganese steel, which consists in quenching the unworked steel at a temperature above its point of recrystallization to rapidly reduce the temperature of said steel to a point where no further structural 100 changes take place, and reheating to a rolling temperature, substantially as described.

2. The process of treating a manganese steel ingot, which consists in quenching the ingot at a temperature above its point of 105 recrystallization to rapidly reduce the temperature of said steel to a point where no further structural changes take place, and reheating said ingot to a rolling temperature, substantially as described.

3. The process of treating a manganese steel ingot, which consists in stripping the

ingot, and quenching said ingot before its temperature has fallen below approximately 750° C. to rapidly reduce the temperature of said steel to a point where no further structural changes take place, substantially as described.

4. The process of treating a manganese steel ingot, which consists in stripping the ingot, quenching said ingot before its temperature has fallen below approximately

750° C. to rapidly reduce the temperature of said steel to a point where no further structural changes take place, and reheating to a temperature of approximately 1175° C., substantially as described.

CHARLES G. OSBORNE.

Witnesses:

W. C. Post,  
D. V. MEDALIE.